

## UNITED STATES PATENT OFFICE

2,346,077

## METHOD OF TONING PHOTOGRAPHIC IMAGES

Howard A. Miller, Rochester, N. Y., assignor to  
Eastman Kodak Company, Rochester, N. Y., a  
corporation of New Jersey

No Drawing. Application November 25, 1941,  
Serial No. 420,369

11 Claims. (Cl. 95—88)

This invention relates to a method for toning photographic images.

It is well known that photographic silver images may be converted to a form in which they can be toned with sulfur compounds such as sodium sulfide to vary the color of the image. The dominant hue of the silver sulfide image formed in this way or of similarly formed silver selenide or telluride images varies with the nature of the photographic emulsion employed. Frequently the print yields a tone which is too purple or cold and it is desirable to produce an image having a warmer tone.

It is, therefore, the principal object of the present invention to provide a method for producing a warm toned photographic image. A further object is to provide a method for regulating the tone of the photographic image in the "indirect" process of sulfide toning. Other objects will appear from the following description of my invention.

These objects are accomplished by treating the photographic image to be toned in a bath containing thioacetamide or a thiourea as a toning agent and also containing as a restraining agent one or more of various sulfur compounds.

The restraining agents used according to my invention include thibarbituric acid, rhodanine, substituted thiohydantoins such as 1-acetyl-2-thiohydantoin and 1-benzoyl-2-thiohydantoin, dialkyl-substituted thioureas, thiobenzanilide and thioacetanilide. These restraining agents are used in amounts varying from 0.1 gram to 2 grams or more per liter of the toning solution.

My invention is preferably used in the "indirect" process of sulfide toning photographic prints. In this process a developed and fixed photographic image is bleached in a solution such as ferricyanide and bromide or potassium permanganate and hydrochloric acid which converts the silver image to a silver salt and is then washed and toned in a solution of a sulfide or other sulfur toning agent (Neblette "Photography Principles and Practice," 2nd edition, 1930, page 440).

According to the preferred embodiment of my invention, after treatment of the silver image with the bleaching solution of ferricyanide and bromide, it is toned in a sulfur toning bath consisting of an alkaline solution of thioacetamide or a thiourea containing one of the restraining agents specified above. By the addition of increasing concentrations of these restraining agents to the toning bath, prints were produced

ranging from a cold "platinum" tone to a very yellow brown image.

To illustrate my invention more specifically, a typical toning procedure will be described.

After exposure, development and fixing of photographic prints on paper, the silver images were bleached in a solution of the following composition:

10 Potassium ferricyanide \_\_\_\_\_ grams 20  
Potassium bromide \_\_\_\_\_ do 20  
Water to \_\_\_\_\_ liter 1

This bleach bath converted the silver images to a silver salt or salts capable of being toned.

15 The prints were then rinsed and a check print was treated in a solution of the following composition:

18 Thioacetamide \_\_\_\_\_ grams 1  
Borax \_\_\_\_\_ do 10  
20 Water to \_\_\_\_\_ liter 1

The tone produced by this treatment was the typical cold tone resulting from sulfide toning without the use of a restraining agent.

25 Toning solutions were made up containing various restraining agents and having the following composition:

28 1. Thioacetamide \_\_\_\_\_ grams 1  
30 Borax \_\_\_\_\_ do 10  
Thiobarbituric acid \_\_\_\_\_ do 0.1 to 2  
Water to \_\_\_\_\_ liter 1  
35 2. Thioacetamide \_\_\_\_\_ grams 1  
Borax \_\_\_\_\_ do 10  
Thioacetanilide \_\_\_\_\_ do 0.1 to 2  
Water to \_\_\_\_\_ liter 1  
40 3. Acetyl thiourea \_\_\_\_\_ grams 1  
Sodium carbonate \_\_\_\_\_ do 10  
Thiobarbituric acid \_\_\_\_\_ do 0.1 to 2  
Water to \_\_\_\_\_ liter 1

Upon treatment of the bleached prints in these solutions containing various amounts of the restraining agents, it was found that upon increasing the amount of restraining agent the tone of the prints became warmer until a very yellow brown image was produced with the solutions containing 2 grams per liter of the restraining agent.

50 The toning baths may be used in alkaline solutions such as solutions containing sodium carbonate or borax. Although some of the restraining agents which I propose to use have previously been suggested for use in toning solutions, none of them has any toning action alone in borax

solutions. The restraining agents are intended for use only in conjunction with sulfur toning agents and have no toning action when used alone.

It will be understood that my invention is susceptible of variations which will be apparent to those skilled in the art and that my invention is taken as limited only by the scope of the appended claims.

I claim:

1. The method of restraining cold tones and producing warm tones in toning a photographic silver salt image, which comprises treating the image in an alkaline solution of a toning agent selected from the group consisting of acetyl thiourea and thioacetamide, containing a restraining agent selected from the group consisting of thiobarbituric acid, rhodanine, 1-acyl-2-thiohydantoins, dialkyl thioureas, thiobenzanilide, and thioacetanilide.

2. The method of restraining cold tones and producing warm tones in toning a photographic silver salt image, which comprises treating the image in a borax solution of a toning agent selected from the group consisting of acetyl thiourea and thioacetamide, containing a restraining agent selected from the group consisting of thiobarbituric acid, rhodanine, 1-acyl-2-thiohydantoins, dialkyl thioureas, thiobenzanilide, and thioacetanilide.

3. The method of restraining cold tones and producing warm tones in toning a photographic silver salt image, which comprises treating the image in a borax solution of thioacetamide containing thiobarbituric acid.

4. The method of restraining cold tones and producing warm tones in toning a photographic silver salt image, which comprises treating the image in a borax solution of thioacetamide containing thioacetanilide.

5. The method of restraining cold tones and producing warm tones in toning a photographic silver salt image, which comprises treating the image in a sodium carbonate solution of acetyl thiourea containing thiobarbituric acid.

6. The method of producing a warm-tone photographic image which comprises exposing, developing and fixing a sensitive silver halide layer, treating the layer with a ferricyanide and bromide solution to form a silver salt image, and then toning said silver salt image in an alkaline solution of a toning agent selected from the group consisting of acetyl thiourea and thioacet-

amide, containing a restraining agent selected from the class consisting of thiobarbituric acid, rhodanine, 1-acyl-2-thiohydantoins, dialkyl thioureas, thiobenzanilide, and thioacetanilide.

7. The method of producing a warm-tone photographic image which comprises exposing, developing and fixing a sensitive silver halide layer, treating the layer with a ferricyanide and bromide solution to form a silver salt image, and then toning said silver salt image in a borax solution of a toning agent selected from the group consisting of acetyl thiourea and thioacetamide, containing a restraining agent selected from the class consisting of thiobarbituric acid, rhodanine, 1-acyl-2-thiohydantoins, dialkyl thioureas, thiobenzanilide, and thioacetanilide.

8. The method of producing a warm-tone photographic image which comprises exposing, developing and fixing a sensitive silver halide layer, treating the layer with a ferricyanide and bromide solution to form a silver salt image, and then toning said silver salt image in a borax solution of a toning agent selected from the group consisting of acetyl thiourea and thioacetamide, containing thiobarbituric acid.

9. The method of producing a warm-tone photographic image which comprises exposing, developing and fixing a sensitive silver halide layer, treating the layer with a ferricyanide and bromide solution to form a silver salt image, and then toning said silver salt image in a borax solution of thioacetamide containing thiobarbituric acid.

10. The method of producing a warm-tone photographic image which comprises exposing, developing and fixing a sensitive silver halide layer, treating the layer with a ferricyanide and bromide solution to form a silver salt image, and then toning said silver salt image in a borax solution of thioacetamide containing thiobenzanilide.

11. The method of restraining cold tones and producing warm tones in toning a photographic silver salt image, which comprises treating the image in a sodium carbonate solution of a toning agent selected from the group consisting of acetyl thiourea and thioacetamide, containing a restraining agent selected from the group consisting of thiobarbituric acid, rhodanine, 1-acyl-2-thiohydantoins, dialkyl thioureas, thiobenzanilide, and thioacetanilide.

HOWARD A. MILLER.